

July 26, 1960

A. BEERBOWER ET AL  
CONTINUOUS GREASE MANUFACTURE USING COATED FREE-FLOWING  
ALKALI METAL SAPONIFYING AGENT  
Filed March 26, 1956

2,946,751



Allan Beerbower  
William H. Meyer

Inventors

By *E.J. Brenner* Attorney

1

2,946,751

**CONTINUOUS GREASE MANUFACTURE USING COATED FREE-FLOWING ALKALI METAL SAPONIFYING AGENT**

Alan Beerbower and William H. Meyer, Baltimore, Md., assignors to Esso Research and Engineering Company, a corporation of Delaware

Filed Mar. 26, 1956, Ser. No. 573,677

5 Claims. (Cl. 252—40)

This invention relates to a new and improved method for the manufacture of metal base oil slurries. More particularly, the invention relates to a process for continuously making alkali metal oil slurries useful in the preparation of lubricating grease compositions and lubricating grease soap concentrates.

In the prior art there have been many attempts to devise effective continuous methods for the manufacture of lubricating grease compositions. There have also been several attempts to directly utilize the essential ingredients such as the saponifying agent, the saponifiable material and the base oil. In U.S. Patent No. 1,912,001 to Lauer an aqueous solution of the saponifying agent was first prepared and then metered in by a pump to the grease-making process. The Lauer process is restricted to the use of sodium hydroxide as no other grease-forming alkali metal base is sufficiently water soluble to avoid the inclusion of very large amounts of water into the grease-making system. In order to obtain a solution of lithium hydroxide, for example, about nine parts of water are required for each part of lithium hydroxide. Thus, a heavy dehydration load is imposed on the subsequent grease-making steps. Another method proposed for the direct utilization of the saponifying agent involved the feeding of dry, powdered metal base by means of a vibratory meter. This latter method is, however, limited to free-flowing powders, such as lime. Alkali metal bases, on the other hand, are not free-flowing powders, since they are hygroscopic in nature and readily absorb moisture from the atmosphere. Consequently, alkali metal bases become adhesive and coalesce and will not flow freely when utilized, for example, after storage or in a vibratory meter feed system.

In accordance with the present invention, a method has been found whereby alkali metal saponifying agents can be utilized directly in continuous grease manufacture without using it to preform the soap thickener or in the form of an aqueous solution. Broadly, the invention comprises rendering alkali metal bases non-hygroscopic and free-flowing by coating them with a dry hydrophobic powder which will be acceptable in the finished grease composition. The coated alkali metal bases may then be used directly in a continuous grease manufacturing operation. Though this method is particularly adapted for continuous grease manufacture, it may also be employed in semi-continuous or batch processes.

The alkali metals contemplated in this invention include sodium and lithium. These alkali metals may be employed in the form of hydroxides, oxides, and carbonates. Finely divided, powdered or flaked alkali metal bases are utilized in preparing the oil slurries of the invention. The particle size will generally be between about 20 mesh and 4 mesh, though flakes up to  $\frac{1}{2}$  inch diameter may be used.

The dry, hydrophobic coating powder may be the alkaline earth metal bases such as calcium hydroxide. The particles must be considerably smaller than those of the alkali base to provide good coating, preferably at most

2

0.02 times the diameter and as low as 0.001 times the diameter. The size will range from 30 millimicrons to 100 mesh, preferably about 1 micron to 200 mesh.

In the preferred embodiment of the invention, lithium hydroxide is the alkali metal base and hydrated lime, i.e. calcium hydroxide, is the dry, powdery coating material. Generally, about 50 to 99 wt. percent, preferably about 60 to 75 wt. percent, of the alkali metal base will be employed in conjunction with about 1 to 50 wt. percent, preferably about 25 to 40 wt. percent, of the hydrophobic coating material. The amount will depend on the particle size ratio in that enough coating material must be used to provide a more or less continuous coating.

The oil used both in making the saponifying agent slurry and in formulating the finished grease composition may be any of the mineral, vegetable, animal or synthetic lubricating oils known to the art. In general, these lubricating oils should have a viscosity of about 50 to 2000 S.U.S. at 100° F. and about 35 to 200 S.U.S. at 210° F., an ASTM pour point of about +20 to  $-75$ ° F., a flash point of about 350° to 650° F., and a viscosity index of about 0 to 165. Conventionally refined mineral lubricating oil derived from paraffinic, naphthenic or mixed base crudes are preferred. The saponifying agent-oil slurry of the invention will contain about 40 to 70 wt. percent, preferably about 45 to 50 wt. percent, of the lubricating oil base stock. The proportion of lubricating oil in the finished grease composition will ordinarily be about 75 to 95 wt. percent, preferably about 80 to 90 wt. percent.

The synthetic lubricating oils useful in the invention include esters of monobasic acids (e.g. an ester of C<sub>8</sub> Oxo alcohol with C<sub>8</sub> Oxo acid, an ester of C<sub>13</sub> Oxo alcohol with octanoic acid, etc.), esters of dibasic acids (e.g. di-2-ethyl hexyl sebacate, di-nonyl adipate, etc.), esters of glycols (e.g. C<sub>13</sub> Oxo acid diester of tetraethylene glycol, etc.), complex esters (e.g. the complex ester formed by reacting one mole of tetraethylene glycol with two moles of sebacic acid and two moles of 2-ethyl-hexanol, a complex ester formed by reacting one mole of tetraethylene glycol, one mole of C<sub>8</sub> Oxo alcohol, one mole of adipic acid, and one mole of C<sub>8</sub> Oxo acid, etc.), esters of phosphoric acid (e.g. the ester formed by contacting three moles of the mono-methyl ether of ethylene glycol with one mole of phosphorous oxychloride, etc.), hydrocarbon oils (e.g. the polymer of chlorotrifluoroethylene containing twelve recurring units of chlorotrifluoroethylene), alkyl silicates (e.g. methyl polysiloxanes, ethyl polysiloxanes, methyl-phenyl polysiloxanes, etc.), sulfite esters (e.g. ester formed by reacting one mole of sulfur oxychloride with two moles of the methyl ether of ethylene glycol, etc.), carbonates (e.g. the carbonate formed by reacting C<sub>8</sub> Oxo alcohol with ethyl carbonate to form a half ester and reacting this half ester with tetraethylene glycol), mercaptals (e.g. the mercaptal formed by reacting 2-ethyl hexyl mercaptan with formaldehyde), formals (e.g. the formal formed by reacting C<sub>13</sub> Oxo alcohol with formaldehyde), polyglycol type synthetic oils (e.g. the compounds formed by condensing butyl alcohol with fourteen units of propylene oxide, etc.), or mixtures of the above in any proportions.

The slurry may also, if desired, be made with any volatile non-solvent for the alkali and coating which may be removed during subsequent steps. Ketones, alcohols, ethers, etc. may be employed for this purpose.

The saponifiable material useful in preparing the soap thickeners of the invention may be any of the naturally occurring or synthetic fats or fatty acids. Examples of these materials include aliphatic saturated or unsaturated fatty acids having Iodine Numbers within the range of 0 to 150 and having about 12 to 30, preferably about 14 to 22, carbon atoms per molecule, such as lauric, myristic,

palmitic, stearic, 12-hydroxy stearic, 9,10-dihydroxy stearic, behemic, myristoleic, palmitoleic, oleic, linoleic, cottonseed oil fatty acids, palm oil fatty acids, hydrogenated fish oil fatty acids, lignoceric, ricinoleic, erucic acids and their mixtures and/or their glycerides such as lard, beef, rapeseed, palm, menhaden, herring, castor oils, etc. Ordinarily, about 5 to 20 wt. percent, preferably about 8 to 12 wt. percent, of saponifiable fats or fatty acids will be employed in preparing the finished lubricating grease compositions.

In general, the saponifying agent or metal base slurry of the invention is prepared by first mixing the alkali metal base with the desired proportion of the hydrophobic coating material, e.g. hydrated lime. Any of the known powder mixers may be employed to blend the alkali metal base and the dry coating powder. The powder may, for example, be added intermittently as in a Patterson-Kelly Dry Blender. Alternatively, the dry ingredients may be dumped more or less continuously into a mixing trough fitted with an agitator such as ribbon mixer. A continuous tube or ball mill may also be employed. Any of the mixing devices used must have a sufficient volume to "average" the composition of the mixed powders after charging the separate ingredients. The product may be used immediately or stored for as much as a year without deterioration.

The coated alkali metal base is then fed to a vibratory feed meter or a similar type device so that the flow of material can be controlled within about  $\pm 1/2\%$  of the desired rate. The coated alkali metal base is fed to a slurry mixer, which may be open top and relatively small but which is adapted for continuous operation. A metered stream of the oil dispersant is charged to the slurry mixer at the same time, and a slurry of the alkali metal base and the oil is formed by continuous stirring. The resulting slurry may then be either stored or fed to the subsequent grease-making steps by means of a synchronized metering pump or a flow controller. In some instances the slurry may tend to settle in the lines due to the presence of lumps of the alkali metal base. This may be readily prevented by adding a small portion of fatty acid material to the oil stream or directly to the slurry mixer in order to form a sufficient amount of soap which will suspend the alkali metal base in the oil. Ordinarily, only about 0.5 to 5 wt. percent, preferably about 0.5 to 1.0 wt. percent, based on the alkali metal oil slurry, of the fatty acid material need be employed. However, a preferred alternative to this method of stabilizing the suspension of the alkali metal base in the oil involves recycling about 3 to 15 wt. percent, preferably about 5 to 10 wt. percent, based on the slurry, of the finished grease composition to the slurry mixer.

As previously noted, the alkali metal base-oil slurry prepared in accordance with this invention may be utilized in the preparation of any lubricating grease composition wherein alkali metal bases may be employed as the saponifying agent. It is important, of course, that the hydrophobic coating material be acceptable in the final grease composition. In the preferred embodiment the alkali metal base is lithium hydroxide and the dry coating powder is calcium hydroxide. The resulting alkali metal base oil slurry can be utilized in the preparation of lithium-calcium soap thickened greases, having a mol ratio of lithium soap to calcium soap within the range of about 2:1 to 8:1. These particular grease compositions are disclosed in detail in U.S. Patent Nos. 2,641,577 and 2,646,401.

Other grease compositions wherein the alkali metal base-oil slurry of the invention may be utilized include the mixed base and complex soap-salt thickened lubricating grease compositions described in chapters 15 and 16, respectively, of Boner's "Manufacture and Application of Lubricating Greases" (Reinhold Publishing Corp., New York, 1954).

In order to more clearly set forth the invention, reference is now made to the accompanying drawing, which

is a flow diagram illustrating a method of preparing the metal base oil slurries and the finished grease compositions of this invention. It is to be understood, however, that modification as to equipment, its arrangement, the type of materials and their proportions can be resorted to without departing from the concept of this invention.

Referring now to the drawing, ribbon mixer 1 is supplied with a hygroscopic alkali metal base powder via line 9 and a dry, hydrophobic powder via line 10 in a continuous manner. The powders are thoroughly mixed together in ribbon mixer 1, and the resulting mixture passed via line 11, vibratory feed meter 2 and line 12 into slurry mixer 3. Simultaneously, an oil dispersant is charged to slurry mixer 3 via line 14 from oil reservoir 5, and the resulting mixture thoroughly agitated to produce a metal base oil slurry. The slurry is continuously removed from slurry mixer 3 via line 15 and slurry pump 16 either to storage via line 25 or to grease cooker 4. If the metal base oil slurry is passed to grease cooker 4, the desired proportion of lubricating oil is simultaneously pumped into grease cooker 4 from oil reservoir 5 via line 17. Fatty acid material is also charged to grease cooker 4 from the fatty acid tank 6 via line 18. Sufficient heat is supplied to cooker 4 to heat the resulting mixture to a grease-making temperature within the range of about 225° to 350° F., preferably about 300° to 325° F., though the temperature required will depend upon the various grease-making ingredients employed. If desired, the water liberated by the reaction in cooker 4 can be vaporized and vented via line 26.

After saponification of the fatty material has been completed in cooker 4, the resulting grease mixture is withdrawn via line 21 and passed to cooler 7, which may be any one of the conventional coolers employed in the grease manufacture art. In general, the grease will be cooled to a temperature within the range of about 100° to 150° F. If desired, the cooled grease may then be homogenized at high rates of shear within the range of about 50,000 to 500,000 reciprocal seconds in such milling or homogenizing devices as a Morehouse mill, Charlotte mill, ink mill, Manton-Gaulin homogenizer, etc. Where it is desirable, conventional lubricating grease additives may be added to the grease prior to homogenization via line 24. Examples of such additives include oxidation inhibitors, corrosion and rust inhibitors, extreme pressure agents, metal deactivators and the like.

As previously discussed, should the metal base-oil slurry tend to settle in the lines, this can be prevented by charging a small amount of the fatty acid material directly to slurry mixer 3 from fatty acid tank 6 via line 19 or to oil stream 14 via lines 19 and 20. However, the preferred method of stabilizing the metal base in the oil involves supplying a small portion of the finished grease composition from the homogenizer via lines 23 and 13.

The following examples are presented to illustrate the preparation of a metal base-oil slurry and a finished grease composition manufactured according to the process of this invention.

#### Example I

60 A metal base-oil slurry was prepared from the following ingredients:

|                                          | Wt. percent |
|------------------------------------------|-------------|
| Lithium hydroxide monohydrate            | 23.67       |
| Hydrated lime (200 mesh)                 | 13.33       |
| Lithium-calcium grease <sup>1</sup>      | 5.00        |
| Mineral lubricating oil 70 SUS @ 210° F. | 58.00       |
|                                          | 100.00      |

<sup>1</sup> Formulation, wt. percent:

|                                              |        |
|----------------------------------------------|--------|
| Animal fatty acid                            | 12.60  |
| Lithium hydroxide monohydrate                | 1.50   |
| Hydrated lime                                | 0.70   |
| Mineral lubricating oil 70, S.U.S. @ 210° F. | 85.20  |
|                                              | 100.00 |

75 The slurry was prepared by mixing the lithium hydroxide monohydrate and the hydrated lime in a Patterson

Kelly Blender for about 15 minutes. The resulting mixed powder was then metered on an Omega Machine Feeder to a Stratco Contactor with the mineral lubricating oil and the lithium-calcium base grease. The resulting slurry was stable in storage, showing no separation of oil or sediment in one month at 80° F. In consistency it was sufficiently fluid to be readily poured or pumped. Its viscosity, determined on a Brookfield Viscosimeter (#2 Spindle, 10 r.p.m.), was as follows:

| Temperature, ° F.: | Viscosity, poises |
|--------------------|-------------------|
| 77                 | 8.4               |
| 125                | 5.2               |
| 175                | 2.9               |

*Example II*

The alkaline slurry of Example I was metered by a screw type pump at 6.9 lb./min., 200° F. and 100 p.s.i.g. while fatty acid was metered by a gear pump at 15.3 lb./min., 180° F. and 100 p.s.i.g. The streams joined in a Lancaster Disperser driven at 3500 r.p.m. The soap mixture, then at 260° F., was led through a scraped surface heater, leaving at 296° F. Oil at a rate of 77.8 lb./min., 135° F. and 100 p.s.i. was metered in by a gear pump and mixed with the soap in a second disperser. The resulting grease at 235° F. was passed through a pressure reducing valve and dehydrated in a Cornell Homogenizer at 21" vacuum cooled to 135° F. and milled in a Charlotte Colloid Mill at .015" clearance. It had a worked penetration of 270, passed the A.S.T.M. Wheel Bearing Test, and was smooth and unctious in texture.

It will be further understood that the invention is not necessarily limited to the specific materials and operating conditions of the foregoing examples. These materials and conditions may be varied within the limits indicated in the general portions of the specification.

What is claimed is:

1. In a process for preparing a lubricating grease composition comprising feeding an alkali metal base to a mixing zone, simultaneously feeding a lubricating oil dispersant to said mixing zone to obtain an alkali metal base oil slurry, mixing said slurry with additional lubricating oil dispersant and a grease-thickening proportion of a saponifiable material, heating the resulting mixture to a grease-forming temperature, dehydrating and then cooling to obtain said lubricating grease composition, the improvement which comprises maintaining said alkali metal base free-flowing by thoroughly mixing it with a dry, alka-

line earth metal base powder sufficient in amount to coat said alkali metal base.

2. A continuous process for preparing a lubricating grease composition which comprises forming an intimate mixture consisting essentially of dry finely divided lithium hydroxide and dry finely divided calcium hydroxide in a separate mixing zone to obtain non-hygroscopic lithium hydroxide coated with said calcium hydroxide, feeding said coated lithium hydroxide to a second mixing zone, 10 charging a dispersing proportion of a lubricating oil to said second mixing zone to obtain a metal base oil slurry, then admixing said slurry with additional lubricating oil and a grease-thickening proportion of a high molecular weight carboxylic acid having from about 12 to 30 carbon atoms per molecule, heating the resulting mixture to a grease-forming temperature, dehydrating and then cooling to obtain said lubricating grease composition.
3. The process of claim 2 wherein a small proportion of said high molecular weight carboxylic acid is charged to said second mixing zone.
4. The process of claim 2 wherein a small proportion of said finished lubricating grease composition is charged to said second mixing zone.
5. The process of claim 2 wherein the finished lubricating grease composition contains a mol ratio of lithium to calcium soap within the range of about 2:1 to 8:1.

References Cited in the file of this patent

UNITED STATES PATENTS

|    |           |                      |                |
|----|-----------|----------------------|----------------|
| 30 | 143,430   | Wyle                 | Oct. 7, 1873   |
|    | 318,044   | Semper               | May 19, 1885   |
|    | 1,342,148 | Armstrong            | June 1, 1920   |
|    | 1,601,898 | Wiley et al.         | Oct. 5, 1926   |
| 35 | 1,872,026 | Carey                | Aug. 16, 1932  |
|    | 2,031,972 | Moser                | Feb. 25, 1936  |
|    | 2,207,737 | Vissert Hooft et al. | July 16, 1940  |
|    | 2,296,689 | Soderberg            | Sept. 22, 1942 |
|    | 2,383,906 | Zimmer et al.        | Aug. 28, 1945  |
| 40 | 2,470,214 | Egan                 | May 17, 1949   |
|    | 2,488,485 | Winternitz           | Nov. 15, 1949  |
|    | 2,514,331 | Morway               | July 4, 1950   |
|    | 2,589,108 | Mark                 | Mar. 11, 1952  |
| 45 | 2,625,508 | Stross               | Jan. 13, 1953  |
|    | 2,629,652 | Schechter et al.     | Feb. 24, 1953  |
|    | 2,641,577 | O'Halloran           | June 9, 1953   |
|    | 2,684,947 | Kramer               | July 27, 1954  |